

Dec. 22, 1953

H. E. TSCHOP ET AL

2,663,631

REDUCTION OF OXIDES

Filed Aug. 27, 1949

6 Sheets-Sheet 1

COMPARATIVE FLOW-SHEETS FOR PRODUCTION OF METAL  
FROM METALLIC OXIDES

FLOW SHEET "A"  
OLD PROCESS



FLOW SHEET "B"  
NEW PROCESS



Fig. 1.

BY

*C. Dr. Weller*  
ATTORNEY

INVENTORS  
HARRY EDWIN TSCHOP  
JOSEPH EDWIN CARTER  
CHARLES BRUCE GOODRICH

Dec. 22, 1953

H. E. TSCHOP ET AL

2,663,631

REDUCTION OF OXIDES

Filed Aug. 27, 1949

6 Sheets-Sheet 2

SCHEMATIC DIAGRAM OF REACTION ZONES  
IN ANNULAR MUFFLE



Dec. 22, 1953

H. E. TSCHOP ET AL

2,663,631

REDUCTION OF OXIDES

Filed Aug. 27, 1949

6 Sheets-Sheet 3



INVENTORS  
HARRY EDWIN TSCHOP  
JOSEPH EDWIN CARTER  
CHARLES BRUCE GOODRICH

BY

*C. A. Weller*  
ATTORNEY

Dec. 22, 1953

H. E. TSCHOP ET AL

2,663,631

REDUCTION OF OXIDES

Filed Aug. 27, 1949

6 Sheets-Sheet 4



Dec. 22, 1953

H. E. TSCHOP ET AL

2,663,631

REDUCTION OF OXIDES

Filed Aug. 27, 1949

6 Sheets-Sheet 5

*Fig. 6.*



Dec. 22, 1953

H. E. TSCHOP ET AL

2,663,631

REDUCTION OF OXIDES

Filed Aug. 27, 1949

6 Sheets-Sheet 6



## UNITED STATES PATENT OFFICE

2,663,631

## REDUCTION OF OXIDES

Harry E. Tschop, Joseph Edwin Carter, and Charles Bruce Goodrich, Huntington, W. Va., assignors to The International Nickel Company, Inc., New York, N. Y., a corporation of Delaware

Application August 27, 1949, Serial No. 112,774

12 Claims. (Cl. 75—1)

1

The present invention relates generally to an improved process for treating raw oxidic materials containing nickel and/or copper to obtain therefrom high-quality metal. More particularly, the present invention relates to an improved process for partially reducing raw nickel and nickel-copper oxides to obtain a uniformly high metal content in said oxides and then to subsequently directly smelt and refine said partially-reduced oxides to produce finished nickel and nickel alloys containing copper whereby the production of metal from said oxides is greatly simplified and facilitated, to a machine having a novel structure for obtaining controlled partial reduction of said oxides, and to a unique partially-reduced oxide product.

Heretofore, the nickel and nickel-copper bessemer mattes and/or sintered mattes available as raw material for the usual open-hearth furnace, electric-arc furnace, or induction-furnace smelting and refining processes were treated first by roasting the nickel and/or copper-containing mattes to oxides and then by partially reducing the hot oxides with charcoal in an endeavor to obtain a consistently uniform and substantially high metal content in said oxides. In some cases, a double roasting was necessary to obtain a satisfactory elimination of sulfur prior to reducing with charcoal. The reduced nickel or nickel-copper oxides were then used as part of the smelting charge along with charcoal or tar coke in acid open-hearth melting and refining operations. Further processing included either direct casting into pigs or else duplex refining the molten metal from the open hearth in a basic electric-arc furnace before casting into ingots.

Another method of sulfur elimination in the matte-sintering process was developed whereby low-sulfur, raw nickel oxide or nickel-copper oxides containing essentially no free metal were produced, these oxides then being smelted with tar-coke additions to molten metal in gas-fired, batch-type furnaces without preliminary roasting. This method was also unsatisfactory in that reducing gases formed within the charge were diluted with and rapidly removed by the combustion gases. In addition, the coke-oxide mixture was insulating in character and heat penetrated very slowly to the interior portions of the charge. The overall result was a relatively slow reaction which began on the exposed surface of the charge and which proceeded slowly inwardly as the surface layers were reduced and melted away. Furthermore, contaminating ele-

2

ments, such as sulfur, were introduced into the metal by the tar coke and had to be eliminated by subsequent desulfurizing treatments.

The art has long sought a simple, inexpensive method for rapidly reducing oxides to obtain products of controlled composition which could then be directly converted to high-quality metal in a single smelting-refining operation. This problem was not solved by any of the conventional processes employed by or known to the art until the advent of the present discovery. One phase of the problem of reducing the oxides involves obtaining a high concentration of reducing gases in contact with the oxides which is necessary for rapid reduction of the oxides. This condition is attained only when dilution and contamination of the reducing gases by nitrogen and/or combustion gases is avoided. In actual practice, this condition cannot be attained in a blast furnace, 20 a reverberatory-type furnace or a direct-fired rotary kiln. Another phase of the oxide-reduction problem involves high thermal efficiency and excellent heat-transfer characteristics coupled with the employment of inexpensive fuel. The 25 numerous processes which have been employed and which were intended to produce high concentrations of uncontaminated reducing gases in intimate contact with the oxides to be reduced have all been very unsatisfactory from the viewpoint of thermal efficiency, heat transfer and economy. In particular, the conventional methods for producing nickel or nickel-copper alloys from the oxides of these metals have been relatively complicated, time and space consuming and costly. Furthermore, the metal content of 30 the oxides reduced by the prior art methods preparatory to smelting and refining was variable and unpredictable.

Up to the present time, the art has failed to 40 develop a technically efficient and economic process and apparatus which would obtain concomitantly all the foregoing necessary conditions and satisfactorily solve the problem in a practical manner, particularly on an industrial scale to produce commercially acceptable products. 45 The foregoing remarks are especially applicable to the nickel industry where the volumes of materials handled are less than are those handled in the iron and steel industry and where the metallurgical properties of the nickel and nickel-copper oxides, such as sulfur absorption, etc., differ greatly from those of iron and iron oxides. The pressing nature of the problem is 50 attested by the continued experimentation of the Bureau of Mines on oxide reduction processes

which likewise clearly indicates that the problem exists and that it has not yet been satisfactorily solved by others skilled in the art.

It is an object of the present invention to provide a novel process for simply, economically and rapidly producing nickel and nickel-copper alloys from raw oxides containing these metals which comprises as essential features in novel combination a unique operation for obtaining partially-reduced oxides of uniform and consistently high metal content, directly converting said reduced oxides to high-quality metal in a single smelting and refining operation without substantial addition of supplementary reducing agents.

It is another object of the present invention to provide as an essential feature in a novel combination of operations, an operation for obtaining a high degree of controlled partial reduction of nickel and nickel-copper oxides to obtain a product having consistently high and uniform metal contents and containing controlled amounts of highly-active carbon finely dispersed throughout the partially-reduced oxides.

It is a further object of the present invention to provide as an essential feature thereof, a novel operation and a unique, easily controllable, unitary apparatus for producing partially-reduced oxides of controlled composition from raw oxides which utilize relatively inexpensive hydrocarbon gas, such as natural gas, to reduce said oxides with markedly low consumption of said gas by simultaneously combining high thermal efficiency together with high concentrations of uncontaminated reducing gas in contact with the oxides.

The present invention also provides as an important but not essential feature the recovery and recirculation of valuable reducing components from the spent exhaust gas produced in the essential oxide-reduction operation.

It is a further object of the present invention to provide unique, partially-reduced oxide products having uniform and consistently high metal contents and controlled carbon contents.

Other objects and advantages of the invention will become apparent from the following description taken in conjunction with the drawings, in which:

Fig. 1 gives, for purposes of comparison, flow-sheet A illustrating a prior art process for producing nickel-copper alloy ingots and flow-sheet B illustrating the much more simple and economic procedure for obtaining the same results by the present novel process and apparatus;

Fig. 2 schematically depicts in perspective the location and temperatures of the various zones in an annular oxide-reduction muffle embodying the novel structure of apparatus encompassed by the present invention. It is to be appreciated, however, that divisions between the various zones and the various temperature ranges are of necessity arbitrarily shown in Fig. 2 and that in actual operation said divisions are not sharp but tend to blend into each other at the junctions between adjacent zones;

Figs. 3 and 4 are reproductions of macrophotographs at 10 magnifications of two nickel-copper oxide particles, each partially reduced by one of the two embodiments of the essential oxide-reduction operation of the present process. The oxide particle shown in Fig. 3 was partially reduced by employing con-current gas flow and contains only about 0.05% carbon whereas the oxide particle shown in Fig. 4 was partially reduced by employing counter-current gas flow and contains about 3.85% carbon;

Fig. 5 shows a flow-sheet depicting one particular manner of combining the various operations, units of equipment and features of the present invention and, in addition, also includes the optional embodiment in the oxide-reduction operation of recirculation of reducing gases recovered from spent exhaust gases;

Fig. 6 illustrates an elevational view, partly in section, on an annular oxide-reduction muffle which is a preferred embodiment of the present invention; and

Fig. 7 is a detailed section of the annular muffle structure illustrated in Fig. 6.

Generally speaking, the present invention comprises a novel combination of operations involving the rapid, controlled, partial reduction of raw oxides in a special oxide-reduction muffle of novel structure to produce unique partially-reduced oxide products having consistently high and uniform metal contents and controlled contents of finely-dispersed, highly-active carbon which are then directly converted into high-quality metal products by electric or induction-furnace practice without substantial additions of supplementary reducing agents.

Partially-reduced oxides treated by the present novel process are directly melted along with scrap by the usual electric-arc furnace or induction-furnace technique, the conventional practice of preliminary melting in an acid open-hearth furnace, desulfurizing, etc., prior to duplexing the melt in an electric furnace, being omitted. The purpose of conventional preliminary open-hearth smelting prior to refining and finishing in electric furnaces is necessary mainly to obtain a product suitable for electric-furnace refining since oxides reduced by conventional methods have relatively low and variable total metal contents which render these oxides unsuitable for direct electric-furnace smelting and refining.

In order to obtain material suitable for electric-furnace refining, it is necessary that the oxides charged into the electric furnace be high-grade, i. e., of uniformly high total metal content, both from the viewpoint of metallurgical quality and also cost. The quality of reduced oxides produced by the prior art methods is not only relatively lower from the viewpoint of total metal content but also is quite variable in metal content, e. g., the variation usually is from about 78% to about 85% whereas the minimum desirable metal content for direct electric-furnace smelting is at least about 88% total metal content. These factors render preliminary open-hearth melting a necessary operation before electric-furnace refining and deoxidation can be economically and metallurgically feasible. On the other hand, the partially-reduced oxides produced by the present novel process are of sufficiently high and uniform in quality to permit direct smelting, refining and deoxidation by electric-furnace or induction-furnace practice with considerable savings in operating, labor and equipment costs.

In order to clearly demonstrate the marked distinctions and advantages of the present process over conventional processes, two flowsheets are presented in Fig. 1. Flow sheet A shows a typical prior art process and flow sheet B illustrates the much more efficient, simple and economic process embodying the present invention. In Fig. 1, flow sheet A shows the conventional operations for producing cast ingots containing about 70% nickel and 30% copper, such as sold under the trade-mark "Monel," from sintered nickel-cop-

per oxide. Flow sheet B illustrates the present improved process. Identical amounts of scrap and oxide are shown entering each system and 100,000 pounds of the aforesaid nickel-copper alloy as ingots are produced by both systems. The advantages of the present novel process as compared to the production system employing the old practice are readily apparent by comparing the two flow sheets. In the latter, a small amount of tar coke and oxide is placed in the bottom of the electric furnace, mixed with scrap, melted, refined and cast into ingots which comprise approximately 60% of the total tonnage produced. The balance of the oxide is mixed with about 12% tar coke by weight and charged into a gas-fired, open-hearth furnace where it is reduced and melted. The reduction and melting operation in the open-hearth furnace is slow and inefficient since the oxide-coke mixture has very poor heat-transfer characteristics. Reduction with subsequent melting occurs only on the surface of the charge and any reducing gases, e. g., carbon monoxide, formed by the reaction of the coke with the oxide are rapidly diluted with combustion gases and swept out of the furnace, thereby slowing the reducing action and wasting valuable reducing gases. Unrefined molten metal tapped from the open-hearth furnace is desulfurized in the ladle and the sulfur-containing impurities are removed with the slag. Desulfurization is necessary due to sulfur pick-up from the coke which has been added to the oxide in the open-hearth furnace. This product is transferred to an electric furnace for further refining and is then cast into ingots.

In procedures employing the present new process, including the novel oxide-reduction operation, the oxide is partially reduced in the novel oxide-reducing muffle employing counter-current gas flow. The partially-reduced oxide containing a uniform high total metal content and a controlled carbon content is charged directly into the electric furnace, melted, refined and cast into ingots. A very small amount of tar coke, e. g., up to about 1,000 pounds of tar coke, may be added if desired together with the partially-reduced oxide. In this particular case the optimum total metal content in the partially-reduced oxide is about 91% copper plus nickel together with about 1.5% of carbon finely dispersed throughout the reduced oxide particles.

In the present process, both the conventional mixing and the ladle-desulfurizing operations have been eliminated. Furthermore, the duplexing operation, i. e., the combination of open-hearth and electric-furnace operations, has been eliminated, thereby completely avoiding all delays caused by the unequal tap-to-tap times for the two different types of furnaces. Since the oxide partially reduced by the novel oxide-reduction operation is discharged from the muffle with a low-heat content, it can be stored normally and is available for direct charging into the electric furnace at any time without suffering any loss of activity of the contained, deposited carbon. Furthermore, any extra carbon additions (tar coke additions) made in the new system amount to not more than about 15% of the tar coke added during processing by the old system, but even here this small amount of tar coke can be eliminated when employing the new process. Since the tar-coke requirement of the new process is either nil or at the most negligible, the problem of sulfur contamination by tar coke is also negligible. A still further advantage of the new proc-

ess is the fact that the ratio of scrap to partially-reduced oxide in direct electric-furnace smelting can be varied at will over a much wider range than when processing by conventional methods.

The physical properties and the metallurgical quality of the metals and alloys obtained as commercial products as a result of utilizing the process of the present invention is, in every way, comparable to the quality of the metals and alloys obtained by the more costly and more complicated conventional duplex smelting and refining operations.

The novel oxide-reduction operation in the present process employs hydrocarbon gas, e. g., natural gas, to obtain the desired high degree of controlled partial reduction of the raw oxides. It is contemplated that the flow of the gases can either be con-current with or counter-current to the feed of oxide through the reduction muffle, depending on the carbon content desired in the final product. It has been discovered that natural raw gas, e. g., a gas containing generally about 75% to about 95% methane, is particularly applicable in the present process.

In an embodiment of the oxide-reduction operation, the relatively cool, raw, natural gas enters the novel reduction muffle through the port from which the partially-reduced oxide is discharged where it aids in cooling said oxide. As the gas flows counter-currently to the downwardly-moving column of oxide and upwardly into the high-temperature reducing zone, the progressively increasing temperature encountered accelerates the reduction reactions. The novel result is a partially-reduced oxide of high, consistently uniform metal content discharging from one end of the apparatus and exhaust gases, resulting from the partial oxidation of natural gas and containing hydrogen, carbon monoxide, water vapor, carbon dioxide, nitrogen, hydrocarbon gases, etc., discharging from the other end of said apparatus.

The various zones and temperatures occurring within the reduction muffle when employing counter-current gas flow to obtain partially-reduced oxides of controlled composition are schematically illustrated in Fig. 2. The cool raw natural gas 10, upon entering the oxide-discharge port of the reduction apparatus and upon coming into contact with reduced oxide 11 in cooling zone 12, cools said oxide and is in turn preheated. Above the cooling zone, in zone 13, temperatures above about 1000° F., e. g., at about 1100° F. and higher, are obtained and some oxide reduction also continues to take place to some extent in this zone. Carbon is precipitated on and dispersed within the particles of partially-reduced oxide and the remaining gas flows upwardly into regions of progressively increasing temperature containing progressively less reduced oxide while, at the same time, continuously reacting with the unreduced oxide in main reducing zone 14 and in primary reducing zone 15. The carbon which is deposited on the partially-reduced oxide is carried downward with said oxide and, being intimately dispersed on and within the oxide particles (see Fig. 4), provides a most excellent, highly-active, reducing agent for the subsequent electric-arc or induction-furnace direct smelting of the reduced oxide, "operation 19," to produce metal 19a.

The major function of primary reducing zone 15 is to complete the preheating of the oxide to the reduction temperature range, e. g., about 1700° F. to about 1900° F., both by heat supplied by the internal and external heating chambers (see Figs.

6 and 7) of the novel annular muffle and also by absorption of heat from the hot gases progressing upwardly through the oxide bed. The secondary function of zone 15 is to initiate the reduction of the oxide since the gases leaving the reducing zone 14 still possess potential reducing power.

Initial preheating of the entering raw oxide 18 occurs in the zone 16 which is located immediately above the primary reducing zone but which is positioned outside the external heating chamber of the muffle (not shown in Fig. 2). Pre-heating in zone 16 is accomplished mainly by the heat absorbed from the large volume of exhaust gases.

Heat is supplied to zones 12 to 15 by an external heating chamber 24 (Fig. 6), for muffle diameters over about 5 inches by an internal (core-heating) chamber 21 (Fig. 7), and by the exothermic oxide-reducing reactions. In the present oxide-reduction operation, more gas is employed than is theoretically necessary to reduce the oxide to the desired degree of partial-reduction resulting in an overall negative heat balance. Good heat-transfer characteristics in the novel muffle are therefore a necessary feature in obtaining the excellent results of the present process. Excellent heat-transfer characteristics are attained without unduly high temperature gradients in muffles of diameters in excess of 5 inches by employing not only an external heating chamber but also an internal or core-heating chamber. In employing counter-current gas flow, the upward-moving hot gases serve to uniformly and gradually pre-heat the downward-moving oxide and the heat is then returned to the incoming gases by the downward movement of the oxide. The efficiency of heat recovery is indicated by the fact that the temperature of the spent, exhaust gases 17 (Fig. 2) is generally below about 220° F. Oxide pre-heating is not only desirable from the viewpoint of returning otherwise wasted heat to the system but is also desirable from the viewpoint of uniform and gradual preheating of the incoming oxides together with initial reduction of said oxides by gases now having only a relatively small reducing potential. This condition serves to prevent excessive rates of reduction. Excess reduction rates, obtained when raw oxide is quickly exposed to hot, highly-reducing gases may cause sintering or fusion of the reduced oxide which, in turn, would promote bridging in the muffle, thereby preventing or hindering flow of the oxide through the muffle.

The final, partially-reduced oxide product containing finely-dispersed, highly-active carbon has been found to be eminently suitable for subsequent direct melting and refining. Partially reducing, rather than completely reducing, the oxide together with deposition of carbon in the partially-reduced oxide particles permits a much higher production or "throughput" rate for any given size of reduction muffle than can be realized if the oxide is completely reduced and also permits equally rapid conversion to metal in the subsequent melting and refining operations.

Cooling the partially-reduced oxide to at least about 550° F. or lower is not difficult when employing the foregoing particular embodiment of the present process, namely, counter-current flow of gas to oxide. Heat absorbed by the endothermic decomposition of the incoming gas cools the oxide to about 1100° F. with great rapidity. Further heat is absorbed in heating the cool incoming gas up to its decomposition temperature

so that the remaining amount of cooling to the required oxide-discharge temperature is relatively small.

As disclosed hereinbefore, the partially-reduced oxide produced by employing counter-current flow of gas to oxide contains finely-dispersed carbon which can be controlled over a wide range by varying the operational factors. The carbon content can be controlled between about 0.4% and about 4.0% by weight. Certain overall processing requirements, however, may make it desirable to produce partially-reduced oxide containing carbon in amounts lower than about 0.6%. The aforesaid low-carbon reduced oxide is produced by employing con-current flow of gas with oxide wherein more of the carbon deposited on and within the oxide particles is oxidized to carbon monoxide or carbon dioxide than is the case when counter-current gas flow is employed. In this embodiment of the present process, the gas is introduced at the top of the muffle along with the raw oxide and withdrawn at the bottom along with the reduced oxide. The carbon deposits on the oxide particles in the upper part of the main reducing zone and most of the carbon thus deposited oxidizes as it passes downward with the oxide through the balance of the main reducing zone. Carbon content of oxides reduced by this embodiment can be held at values even below about 0.10% by this method, e. g., at about 0.05% or even lower. However, the thermal efficiency of this embodiment of the novel reduction operation is somewhat lower than when employing counter-current gas flow because in counter-current flow the heat of the exhaust gases is almost completely transferred to the cold raw oxide entering the muffle. With con-current flow this heat is lost. Furthermore, with counter-current flow the heat of the hot reduced material is largely used to heat the incoming gas. With con-current flow this heat is lost. In addition to the heat losses, cooling of the reduced material to below its reoxidation temperature in air, e. g., below about 550° F., becomes more difficult when employing con-current flow; and for large furnaces the extension of the annular muffle into the cooling zone from the reducing zone becomes a matter of practical necessity.

For producing partially-reduced oxides most economically for direct melting and refining by electric-furnace practice, it is preferred to employ counter-current flow of gas to oxide because the degree of reduction can be best controlled and carbon is deposited on and precipitated within the final product particles in amounts between about 0.4% and about 4%, preferably between about 1.0% and about 2.0% and more preferably in an amount about 1.5% by weight of the final product. Oxide partially-reduced by con-current gas flow and containing carbon in amounts below about 0.6% usually is not as suitable for direct electric-furnace melting as is oxide reduced by counter-current gas flow and having higher carbon contents. However, under certain circumstances low-carbon partially-reduced oxide may be required, in which case con-current flow of gas with oxide would be the most feasible embodiment of the oxide-reduction operation to employ. However, by proper control of the operational factors of either embodiment, it is possible to secure a uniform and high degree of reduction together with deposition of controlled amounts of highly-active carbon finely dispersed within the partially-reduced oxide particles which will promote rapid and complete melting and re-

fining directly in either electric-arc or induction furnaces.

Figs. 3 and 4 are reproductions of macrophotographs at 10 diameters of cross-sections of two representative copper-nickel oxide particles produced by both embodiments of the novel reduction operation. The partially-reduced oxide particle shown in Fig. 3 contains about 0.05% carbon and was produced by employing con-current flow of gas and oxide. The partially-reduced oxide particle shown in Fig. 4 was produced using the more preferred embodiment of counter-current flow of gas and oxide and contains about 3.85% carbon. The carbon in the particle of Fig. 4 is clearly and visibly dispersed throughout the particle. The dark areas shown in the particle in Fig. 3 are reduced elemental copper together with some etching pits. Very little dispersed carbon is visible in any portion of this oxide particle as compared to the particle of Fig. 4 which contains relatively large amounts of highly-active and well-dispersed carbon.

The finely-dispersed carbon, such as illustrated by Fig. 4, is immediately available to any oxide areas remaining in such particles and at elevated temperatures, such as those encountered in electric furnaces, rapidly reduces the remaining oxide. The present novel reduction muffle is operated according to the present invention at high throughput capacities to produce carbon-bearing, partially-reduced oxides of uniform composition which are equally suitable for subsequent smelting and refining operations in either electric-arc or induction furnaces as completely-reduced oxides.

Evidence that the carbon deposited on and within the reduced oxide particles is highly active as a reducing agent when compared to the prior art tar-coke reducing agent is supplied by the following example:

Two samples of raw copper-nickel oxide of the same initial composition were 86% reduced in the novel reduction muffle. Test Nos. 1 and 1a were reduced by employing concurrent flow of gas and oxide to obtain about 0.16% carbon content in the reduced oxide. Test Nos. 2 and 2a were reduced by employing counter-current flow of gas to oxide to obtain about 1.72% carbon content in the reduced oxide. With the exception of the direction of gas flow relative to feed of oxide, all other conditions were identical. Test Nos. 1 and 2 were then finely comminuted in order to minimize any advantage test No. 2 might possess over test No. 1 due to the excellent carbon distribution in the test No. 2 sample. Test Nos. 1 and 1a were then mixed with tar coke in an amount sufficient to raise the carbon content up to the amount of carbon in test Nos. 2 and 2a (1.72% carbon). All test samples were then heated to 1900° F. in a closed furnace for 15 minutes (ground test Nos. 1 and 2) and for 20 minutes (underground test Nos. 1a and 2a). All samples then were analyzed to determine the percent reduction obtained in each case. The data obtained are given in the following Table I:

Table I

| Test No. | Condition of Sample | Percent C after 86% Reduction | Time at 1900° F. | Percent Reduction at 1900° F. |
|----------|---------------------|-------------------------------|------------------|-------------------------------|
| 1.....   | ground.....         | 0.16                          | Min.             | 92.7                          |
| 1a.....  | not ground.....     | 0.16                          | 20               | 87.7                          |
| 2.....   | ground.....         | 1.72                          | 15               | 97.4                          |
| 2a.....  | not ground.....     | 1.72                          | 20               | 98.7                          |

From the foregoing table, it is evident that counter-current gas flow (test Nos. 2 and 2a), which produced partially-reduced oxides containing relatively large amounts of finely-dispersed active carbon is superior from the viewpoint of percent reduction in a given time at a given temperature to con-current gas flow (test Nos. 1 and 1a). The difference in percent reduction for a given time and temperature is credited to the much greater activity of the finely-dispersed carbon as compared to tar coke. This difference in the relative reducing potential of finely-disseminated carbon compared to tar coke is even more marked in the case of the unground oxides (test Nos. 1a and 2a) and is believed to be due to the added beneficial effect of finer and better carbon dispersion in unground test No. 2a as compared to unground test No. 1a. From the foregoing data presented in Table I, it is apparent that the active, finely-dispersed carbon deposited within and on the particles of partially-reduced oxide is a more active reducing agent than conventional tar coke. Furthermore, the dispersion of this active carbon within the particles produces a marked increase in the rate of reduction of the oxide to metal in subsequent electric-arc or induction-furnace smelting and refining operations as compared to the rate of reduction obtained by employing tar coke as the reducing agent.

Control of the amount of deposited carbon in the oxide particles produced by counter-current gas flow in the range of about 0.4% to 4.0% is exercised by varying the rate of oxide feed, by raising or lowering the furnace temperature and by varying the quantity of excess natural gas used for reduction. Some degree of carbon control below about 0.4% may be accomplished by humidifying the natural gas before its entry into the muffle. Deposition of carbon in amounts above about 4.0% may be accomplished by the addition of heavier hydrocarbon vapors to the natural gas which causes carbon to be deposited on and within the partially-reduced oxides at the lower temperatures occurring at lower levels in the muffle when employing counter-current gas flow. At these lower temperatures the carbon reacts much more slowly with the un-reduced oxide present and is removed from the muffle by the discharging oxide product before any great amount of the carbon is oxidized. If desired, carbon may be deposited in sufficient quantity not only to complete the reduction of remaining oxide on subsequent direct melting and refining but also to provide additional amounts for a carbon melt-down, i. e., to produce metal containing excess carbon. The unique partially-reduced oxide product of the novel reduction operation cannot be formed if reducing agents such as water gas, hydrogen, solid carbon, or any other agent not containing hydrocarbons is employed for reducing the oxide. The presence of hydrocarbons within the muffle is essential if controlled amounts of carbon are to be deposited on and dispersed within the partially-reduced oxide particles.

For overall diameters over about 5 inches, the reduction muffle must have an annular cross-section which permits both internal and external heating. The annular muffle is so constructed that, regardless of capacity, the ratio of heating surface area to effective annular volume is maintained above about 0.4 and preferably above about 0.5. A ratio of heating surface area to annular volume of 0.4 means that there is 0.4 square

inch of heating surface to 1.0 cubic inch of annular volume. In an annular muffle, the ratio of muffle heating area to muffle volume is determined by the width of the annular space, indicated by the letter W in Figs. 2 and 7. For example, 6" O. D.  $\times$  2" I. D., 14" O. D.  $\times$  10" I. D., and 20" O. D.  $\times$  16" I. D. muffles all have an annular width, or width of oxide bed, of 2 inches and each muffle has a surface area to volume ratio of 1.0. In the art it is well known that the terms O. D. and I. D. means outside diameter and inside diameter, respectively. Similarly, if the width W of the annular space is 3 inches, the aforementioned ratio will be 0.67, and if the width is 4 inches, the ratio will be 0.50, etc. Thus, while both heating area and oxide-bed thickness are of primary importance in securing rapid heating of the oxide within the novel annular muffle, both factors may be expressed in terms of the width of the oxide bed. Thus, reducing the width of the annular space decreases the time required to heat the oxide to the desired temperature for reduction.

Another factor which is important in improving heat transfer and which is influenced by the width of the annular space is the velocity of the reducing gas. For example, two tests, i. e., test Nos. 3 and 4, were conducted in two different circular muffles, neither of which contained an internal or core-heating chamber and in which the temperature of the oxide feeding through the muffles was measured at a point on the axis of the muffle near the bottom of zone 13 both before and after the reducing gas was introduced in counter-current flow to the movement of the oxide. The pertinent data for each test are shown in the following table:

Table II

| Data                                         | Test No. 3 | Test No. 4 |
|----------------------------------------------|------------|------------|
| Temp. with No Gas Flow, ° F.                 | 395        | 475        |
| Temp. with Flow, ° F.                        | 1,540      | 980        |
| Relative Velocity of Reducing Gas            | 1.0        | 1.23       |
| Width of Oxide Bed (muffle diameter), inches | 3          | 6          |
| Height of Reducing Zone, inches              | 30         | 63         |
| Time Oxide was in Reducing Zone, minutes     | 28         | 37         |

The very considerable effect of rate of gas flow on heat transfer by convection heating can be clearly seen in each of the above tests. The reduction reactions begin as soon as the gas is turned on and the net heat balance is endothermic when there is an excess input of natural gas, as was the case with the tests shown in Table II. Therefore, the increases in temperature obtained by flowing natural gas through the muffle, as illustrated by the foregoing test data, cannot be attributed to heat released by the reduction reaction since the net heat balance in the system is negative, but must be attributed to the important effect of velocity of gas flow through the muffle. The relative gas velocity in an annular muffle is determined by the width of the annular space and by the height of the reducing zone. In other words, the dimensions of the muffle tube have a very important effect on the efficiency of heat transfer in the muffle. Thus, for any given volume of gas input, the shorter the distance between inside and outside walls of the annular reduction chamber, then the higher the ratio of heating surface area to muffle volume, the shorter the width of the oxide bed through which heat must be transferred, and the greater the velocity of the gas flowing through the oxide bed.

5 Circular, non-annular muffles having an inside diameter in excess of about 5 inches result in heat-transfer characteristics too poor to justify economic commercial operation. The present, novel, annular muffle overcomes this handicap and permits the construction of any desired size of reduction furnace without loss of high heat-transfer characteristics. The width of the annular muffle space (W in Fig. 2) is important from the commercial viewpoint and, for economic operation, this width should not exceed about 5 inches and preferably not exceed about 4 inches, particularly when nickel or nickel-copper oxides are to be treated.

10 The balance of the test data disclosed in the present specification was obtained in or pertains to one of three furnaces, the dimensions and operating data for which are given in Table III. Test Nos. 15 to 26 and 39 to 48, inclusive, were made in a small-scale, non-annular furnace (furnace A), and test Nos. 11 to 14 and 27 to 38, inclusive, were made in a medium-sized, semi-commercial annular furnace (furnace B). Test Nos. 5 to 10, inclusive, were computed for a large-scale furnace of the dimensions of furnace C with the exception that the annular width was varied from 1 to 5 inches. The dimensions, capacities, ratios, etc., of furnaces A, B and C are in the following Table III:

Table III

| Reduction Zone Data                               | Furnace |       |       |
|---------------------------------------------------|---------|-------|-------|
|                                                   | A       | B     | C     |
| Reducing Zone O. D., inches                       | 3       | 6     | 18    |
| Reducing Zone I. D., inches                       | 0       | 2     | 12    |
| Reducing Zone Height, inches                      | 30      | 63    | 135   |
| Width of Oxide Bed, inches                        | 3       | 2.0   | 3.0   |
| Ratio Heating Surface                             | 1.33    | 1.00  | 0.666 |
| Volume                                            |         |       |       |
| Relative Reducing Gas Velocities                  | 1       | 2.46  | 3.75  |
| Oxide Feed Rate, lbs/hr.                          | 40      | 350   | 3,000 |
| Reducing Gas Consumption in Ft. <sup>3</sup> /lb. |         |       |       |
| Oxide                                             | 1.50    | 1.50  | 1.50  |
| Time in Reducing Zone, min.                       | 34.5    | 29.4  | 41.3  |
| Time at Reducing Temp., min.                      | 17.6    | 14.4  | 17.1  |
| Reducing Temp., ° F.                              | 1,700   | 1,900 | 1,900 |

50 Since the reduction muffle of furnace A was only 3 inches in diameter (the width of the oxide bed), it was not necessary to provide this furnace with an internal, core-heating chamber. In this case, the high heating surface to muffle volume ratio, narrow width of oxide bed and a relatively high reducing gas velocity for this ratio and width results in good performance without core heating. In larger furnaces, high efficiency is obtained by employing core-heating means. The foregoing muffles obtain markedly improved results in that there is obtained maximum throughput capacity coupled with unusual and markedly superior heat-transfer characteristics. Another factor controlling the width of the annular muffle space that can be employed is the particle size of the oxide charged, as discussed hereinafter. However, it has been discovered that there is an optimum width of annular muffle space for each specific application of this novel reduction operation and that this width is highly important from the viewpoint of economic practicability. For example, a certain copper-nickel oxide charged into furnace C at a rate of 3000 lbs. per hour will require about 24.2 minutes to reach a temperature of about 1500° F. plus an additional time of about 16 minutes at temperatures between about 1500° F. and about 1900° F. to be reduced about 75%. The data given in following Table IV were

computed for a furnace having the overall dimension of furnace C but with the annular width varied, calculations being based on data obtained on furnace B. These data illustrate the effect of varying the width of the annular muffle space on the time at temperature at a feed rate of 3000 lbs. per hour of oxide in all cases.

Table IV

| Test No. | Muffle Diameter, Inches |        | Width of Annular Space, Inches | Time in Minutes  |                    |                 |
|----------|-------------------------|--------|--------------------------------|------------------|--------------------|-----------------|
|          | Outside                 | Inside |                                | In Reducing Zone | To Reach 1,500° F. | Above 1,500° F. |
| 5        | 18                      | 16     | 1.0                            | 14.8             | 6.6                | 8.2             |
| 6        | 18                      | 14     | 2.0                            | 29.4             | 15.0               | 14.4            |
| 7        | 18                      | 12     | 3.0                            | 41.3             | 24.2               | 17.1            |
| 8        | 18                      | 11     | 3.5                            | 46.6             | 29.1               | 17.5            |
| 9        | 18                      | 10     | 4.0                            | 51.5             | 34.2               | 17.3            |
| 10       | 18                      | 8      | 5.0                            | 56.6             | 46.8               | 9.8             |

From the foregoing data, it may be seen that when the factor of time at reducing temperature is introduced, the commercially practical optimum width of the annular space is not necessarily the minimum width. For example, use of a 1-inch width results in very rapid heating (excellent heat transfer), but the volume of the muffle is so reduced that the total time in the heating zone is less than the 16 minutes required to obtain about 75% reduction. At the other extreme, increasing the width of the annular space above about 5 inches results in such poor heat transfer that the oxide never reaches the desired reduction temperature unless the oxide feed rate is lowered below a commercially acceptable rate. From the foregoing data in Table IV, it is obvious that the width of the annular space should not be more than about 5 inches nor less than about 1 inch, preferably not more than 4 inches nor less than about 2 inches, for practical purposes.

For any given muffle diameter the effect of increasing muffle height is to increase the production capacity of the unit. In addition to the obvious advantage of increasing the length of the reducing zone, an increase in oxide feed rate is obtained which in turn requires an increased flow of reducing gas. This results in higher reducing gas velocities within the muffle which in turn improve the heat transfer characteristics of the process. Increased height is always desirable, the only limiting factor being practical engineering considerations, e. g., initial cost and maintenance cost of excessively high structures, etc.

The maximum particle size that can be treated successfully by the reduction operation of the present process depends mainly upon the effective cross-sectional area of the muffle, i. e., width of oxide bed. For any given area of muffle cross-section, the maximum permissible particle size is that size which will move freely downward under the influence of gravity without mechanical clogging. Thus, for the particular muffle dimensions of furnace C described hereinbefore, a particle size of about 0.75 inch is about the maximum size which can be handled without clogging. However, the preferred maximum particle size in this case is about 0.5 inch since particle sizes larger than about 0.5 inch in average diameter require somewhat slower rates of feed than are commercially feasible in order to allow time for diffusion of the reducing gases into the center of each particle. Consequently, in a fur-

nace of the size of furnace C, the reduction reaction rate decreases appreciably as the particle size increases over about 0.5 inch. However, larger particle sizes can also be successfully reduced provided the dimensions of the annular muffle are also increased to accommodate these larger sizes.

Although the maximum permissible particle size is controlled by the capacity of the muffle to handle the oxide without clogging, it has been discovered that the range of particle sizes of the oxide to be treated by the present process is a very important factor in the successful operation of the process. It has been found that if too great a proportion of the oxide being treated is of too fine a particle size, this fine fraction tends to cake or bridge in the reduction muffle thus blocking the muffle and preventing the oxide from properly feeding through the muffle. To obtain the optimum rate of feed, for instance in a furnace of the dimensions of furnace C, it is preferred that the minimum particle size in the oxide feed be maintained at about 0.1 inch although successful reduction can also be obtained with feeds containing oxide particle sizes down to about 0.05 inch (about 14 mesh) provided the percentage of these fine particles in the feed is not too high, e. g., no more than about 10% by volume of the total feed, and provided that a clean sizing separation at the particle size of about 0.05 inch can be made. In order to allow for screening inefficiency and variations in particle size distribution which can occur in commercial scale operations, screening at about 0.1 inch, e. g., from about 6 to about 8 U. S. standard mesh, is recommended. The preferred range of particle size of about 0.1 inch to about 0.5 inch, as contemplated by the present invention for treatment in a muffle of the type of furnace C, is important from the viewpoint of obtaining the best results. However, good results can be obtained in larger size commercial equipment with wider particle size ranges, e. g., about 0.05 inch to about 0.75 inch, provided that the screening facilities are sufficiently good to obtain clean minimum and maximum particle size separations.

The determination of the actual particle size range to be employed with any particular size of apparatus is dictated by at least three considerations. First, the dimensions and the shape of the muffle are important factors in determining the particle size range that may be employed if mechanical clogging and/or caking is to be avoided. Second, the reduction rate decreases as the particle size increases above about 0.4 to about 0.5 inch, the degree of reduction depending on the shape and porosity of the particles and the copper content of the oxide being treated. Third, the success of the present invention depends on intimate contact of the reducing gases with the oxide particles. Conditions favoring intimate contact between oxide and gas are a uniformly porous oxide bed and as small an oxide particle size as is consistent with porosity of the bed without obtaining caking or bridging in the muffle. When the range of particle size of the oxide is wide, the overall porosity of the bed decreases due mainly to the fact that the finer particles tend to segregate in the interstices between the larger particles, thereby forming dense cakes which prevent free uniform passage of the reducing gases. In this case, the gas will tend to channel through or around the segregated fines; and the result is a lower degree of reduction of

the finer particle sizes as illustrated in following Table V, although normally it would be expected that the finer sizes would experience a higher degree of reduction. Furthermore, the tendency of too fine particles to cake and sinter, thereby clogging the muffle tube, is a further reason why the minimum particle size is important and must be controlled.

For any given set of muffle dimensions having a minimum heating surface area to muffle volume ratio of at least about 0.4, the optimum or permissible maximum and minimum particle size for the particular muffle must be determined by actual test. The muffle cross-section is an important factor and increasing the muffle cross-section, particularly with respect to the width of the oxide bed, not only permits treatment of finer particle sizes but also permits treatment of a larger percentage of fine particles in comparison to the particle size range and minimum particle size permissible for treatment in smaller muffles. Furthermore, the permissible range and distribution of sizes determined for any particular apparatus also controls the percentage of fine particles to be allowed. For instance, if the maximum allowable particle size for a specific apparatus is determined by tests to be about 0.2 inch, the minimum permissible particle size can be as low as about 0.04 inch and the percentage of sizes between 0.04 inch and 0.1 inch can be as high as about 50% of the entire feed.

Another important factor in determining the permissible range and distribution of particle sizes is the reduction temperature employed. Thus, the lower the minimum particle size and/or the higher the percent of the finer sizes which are permissible, the lower is the reduction temperature which can be successfully employed. Thus, for a muffle having the dimensions of furnace C when employing reduction temperatures between about 1800° F. and about 2000° F., e. g., about 1900° F.; it is preferred that the particle sizes be between about 0.05 inch and about 0.5 inch with not more than about 10% of the total feed being in the particle size range of about 0.05 inch to about 0.1 inch.

To illustrate the effect of particle size on the degree of reduction of both nickel oxide (containing only about 5% copper) and nickel-copper oxide (containing about 19% copper), each type of oxide was partially reduced in an annular muffle of the dimensions of furnace B. Four particle size ranges were screened from sample of each type of partially-reduced oxide and the total metal content (percent copper plus nickel) was analyzed in each sample. The comparative data are given in the following Table V:

Table V

| Test No. | Particle Size Range (inch) | Percent Copper plus Nickel in Final Product |                      |
|----------|----------------------------|---------------------------------------------|----------------------|
|          |                            | Ni Oxide (5% Cu)                            | Ni-Cu Oxide (19% Cu) |
| 11.      | 0.371 to 0.524             | 83.7                                        | 91.7                 |
| 12.      | 0.263 to 0.371             | 87.3                                        | 91.9                 |
| 13.      | 0.131 to 0.263             | 86.3                                        | 90.8                 |
| 14.      | 0.065 to 0.131             | 85.2                                        | 90.5                 |

It is to be noted that the maximum yield, measured by the total metal content, for both types of oxide is obtained in the narrow particle size range of 0.263 inch to 0.371 inch which lies approximately in the center of the preferred range of about 0.1 inch to about 0.5 inch. To illustrate

the effect of increasing the particle size range on the degree of reduction, three tests were made on nickel-copper oxide at 1700° F. under similar conditions of time, feed rate, and atmosphere, and in a furnace of the dimensions of furnace A. The data are given in the following Table VI:

Table VI

| Test No. | Particle Size Range (inch) | Percent Copper plus Nickel in Final Product |
|----------|----------------------------|---------------------------------------------|
| 15.      | 0.051 to 0.371             | 89.4                                        |
| 16.      | 0.051 to 0.310             | 91.3                                        |
| 17.      | 0.051 to 0.125             | 92.1                                        |

It is apparent from the foregoing data that the more narrow the range of particle size, the higher is the total metal content and the greater is the degree of reduction of the final partially-reduced product.

In commercial operation and employing apparatus of the dimensions of furnace B, an oxide feed rate of at least about 175 pounds of oxide per hour, preferably about 350 pounds of oxide per hour, is desired. For a muffle of the dimensions of furnace C, the desired oxide feed rate for economic operation is at least about 1500 pounds of oxide per hour, preferably about 3000 pounds of oxide per hour. To obtain these high feed rates and, at the same time, to obtain a final reduced oxide product containing over 88%, preferably over 90%, total metal content, it has been discovered that higher temperatures in the 1500° F. to 2000° F. range, preferably between about 1700° F. and 1900° F., are most beneficial in that the rate of heat transfer is markedly increased and the final product, after treatment in the foregoing temperature ranges, averages between about 90% and 95% total metal content. The following Table VII gives data illustrating the effect of various reduction temperatures upon the reduction of a copper-nickel oxide in a muffle of the dimensions of furnace A, all other operating conditions being maintained substantially constant.

Table VII

| Test No. | Reduction Temp., ° F. | Feed Rate, lbs./hr. | Gas Input, Ft.³/lb. | Final Product, Percent Cu+Percent Ni |
|----------|-----------------------|---------------------|---------------------|--------------------------------------|
| 18.      | 1,100                 | 40.0                | 1.50                | 82.0                                 |
| 19.      | 1,300                 | 39.2                | 1.53                | 86.3                                 |
| 20.      | 1,500                 | 40.3                | 1.47                | 91.6                                 |
| 21.      | 1,600                 | 39.8                | 1.48                | 93.2                                 |
| 22.      | 1,700                 | 39.6                | 1.53                | 93.9                                 |
| 23.      | 1,800                 | 38.3                | 1.52                | 94.6                                 |
| 24.      | 1,900                 | 37.9                | 1.58                | 95.3                                 |

It is to be noted that at substantially the same oxide feed rate and input rate of natural gas, there is a definite increase of total metal content in the partially-reduced oxide product as the temperature is increased. An upper limit of about 2000° F. for the reduction temperature is desirable solely from the view point of apparatus deterioration and is not restricted at this particular maximum value due to any change in the nature of the reduction reactions causing a decrease in the total metal content of the treated product. It is also not desirable that the temperature be lower than about 1500° F. purely from the viewpoint of commercial practicality. For instance, a rate of feed of about 35 to 45 pounds of oxide per hour in a muffle of the dimensions of furnace A and selected to give about 90% to

about 92% total metal content at about 1500° F. does not produce anywhere near this total metal value if treated at 1100° F. since the reduction reaction is much slower at this low temperature. In order to obtain a satisfactory uniform product of the desired high metal content, the feed rate must be reduced to only a fraction of the feed rate when employing temperatures above about 1500° F. The following Table VIII illustrates the feed rates necessary to obtain a satisfactory product at temperatures of 1100° F., 1300° F. and 1500° F. in a muffle of the dimensions of furnace A.

Table VIII

| Test No. | Reduction Temp., °F. | Feed Rate, lbs./hr. | Gas Input, Ft.³/lb. | Final Product, Percent Cu+Percent Ni |
|----------|----------------------|---------------------|---------------------|--------------------------------------|
| 20*      | 1,500                | 40.3                | 1.47                | 91.6                                 |
| 25       | 1,300                | 27.1                | 1.37                | 92.2                                 |
| 26       | 1,100                | 9.6                 | 1.56                | 91.7                                 |

\*Data for test No. 20 is also presented in Table VII.

A most important factor affecting the production rate, i. e., the rate of feed of oxide, for any given set of operating conditions is the copper content in the oxide being treated by the present process. In order to illustrate the effect of copper content in accelerating the feed rate while obtaining satisfactory results, a series of tests were made in a muffle of the dimensions of furnace B in which the oxides contained both nickel and copper but wherein the copper content varied in each test from a low value of 4.8% copper to a high value of 19.2% copper. These various oxides were all reduced at 1900° F. by the novel reduction operation, such as is illustrated by the flow-sheet in Fig. 5, employing the reducing equipment of the preferred design shown in Figs. 6 and 7. The optional gas recovery and recirculation system was not used in these tests.

Table IX

| Test No. | Percent Cu in Raw Oxide | Oxide Feed Rate, lbs./hr. | Reduction Temp., °F. | Reducing Gas Ft.³/lb. oxide | Percent Total Cu+Ni in Reduced Oxide |
|----------|-------------------------|---------------------------|----------------------|-----------------------------|--------------------------------------|
| 27       | 4.8                     | 228                       | 1,900                | 1.58                        | 91.5                                 |
| 28       | 4.9                     | 228                       | 1,900                | 1.58                        | 91.9                                 |
| 29       | 4.9                     | 248                       | 1,900                | 1.49                        | 90.9                                 |
| 30       | 6.1                     | 238                       | 1,900                | 1.41                        | 92.1                                 |
| 31       | 11.2                    | 286                       | 1,900                | 1.43                        | 93.0                                 |
| 32       | 10.7                    | 303                       | 1,900                | 1.58                        | 91.8                                 |
| 33       | 11.2                    | 310                       | 1,900                | 1.39                        | 92.8                                 |
| 34       | 11.2                    | 331                       | 1,900                | 1.38                        | 91.8                                 |
| 35       | 19.2                    | 285                       | 1,900                | 1.68                        | 94.8                                 |
| 36       | 19.2                    | 302                       | 1,900                | 1.53                        | 92.2                                 |
| 37       | 19.2                    | 397                       | 1,900                | 1.51                        | 91.5                                 |
| 38       | 19.2                    | 421                       | 1,900                | 1.42                        | 92.3                                 |

It is to be noted that the "throughput" or production rate for the low-copper oxide, i. e., rate of feed of oxide in pounds per hour, is roughly only about 55% of the feed rate for the high-copper oxide and that a slightly lower total metal content is obtained in the final partially-reduced low-copper oxide product. In test Nos. 29 and 35, illustrating a wide difference in copper content (4.9% and 19.2% copper, respectively) for nearly equal feed rates (248 and 285 lbs./hr., respectively), the respective total metal contents show a 3.9% difference in favor of the high-copper oxide in spite of the fact that the high-copper oxide feed rate was somewhat faster. This indication of a slower reaction rate for the reduction of low-copper oxide as compared to the

reaction rate for the reduction of high-copper oxide is believed to be due to the relatively low copper content in the nickel oxide and does not appear to be due to any differences in the porosity of the oxide particles since the difference in porosity between the two types of oxide is practically nil.

In employing the novel muffle in the present process to obtain a partially-reduced nickel or nickel-copper oxide product for direct smelting and refining by electric-furnace practice, the most important requirement is that the partially-reduced oxide be uniform in total metal and carbon contents rather than that the total metal content be very high, although the latter is also very desirable. In other words, it is more important that the degree of partial reduction be controlled to produce a consistently uniform metal content rather than to attempt to more completely reduce the oxide to obtain very high total metal contents. Thus, a degree of partial reduction between about 65% and about 75% (about 90% to about 92% total copper plus nickel content) is much more desirable from the viewpoint of the commercial control of subsequent smelting operations than is a higher degree of reduction which varies between about 75% and about 95% (about 92% to about 96% total copper plus nickel). The desired uniformity of product having reductions in the latter higher range, e. g., from 92% to 96% copper plus nickel, can be obtained at the expense of a lowered "throughput" capacity, particularly for reductions in excess of about 85% (about 94% copper plus nickel). However, it is technically possible to obtain any desired degree of reduction with the reduction operation and apparatus. Degrees of reduction up to about 85% or 90% are obtainable in one single passage of the oxide through the reduction muffle. To obtain still higher reductions, two or more passages of the oxide through the reduction muffle are usually required. Nevertheless, for any given muffle, degrees of reduction in excess of about 75% tend to decrease the "throughput" capacity more and more rapidly as the degree of reduction is increased. Therefore, the optimum degree of reduction in any particular situation depends in large part upon the contemplated subsequent processing operations and also upon the economics of that particular situation.

The metal content of the raw or sintered nickel and nickel-copper oxides such as contemplated for treatment by the present process usually is about 75% to about 80%, essentially all of which is combined. As the oxides are reduced, free or uncombined metal is formed in increasing amounts. However, where values for total metal content of the final product are given in the present specification, it is not meant that these values represent free or uncombined metal but represent free metal plus remaining combined or oxidized metal. Thus, for a reduction of about 75% which is equivalent to a total metal content of about 92%, the free metal content of the final reduced product is about 69%, the balance being combined metal.

Fig. 5 is a flow sheet illustrating the preferred overall process embodying the present invention employing countercurrent flow of natural hydrocarbon gas to oxide to obtain a partially-reduced oxide which is then directly smelted and refined to produce a high-grade metal product. As an embodiment of this preferred overall process, it is contemplated that the partially-spent exhaust

gases can be treated for the separation of reducing components from non-reducing components in the exhaust gases, e. g., the separation of hydrogen, carbon monoxide and hydrocarbon from carbon dioxide, water vapor and possibly nitrogen. The partially-spent exhaust gases can be treated for recovery of hydrogen, carbon monoxide, hydrocarbons, carbon dioxide, etc., in a recovery system such as indicated within the area bounded by dotted lines in the flow-sheet shown in Fig. 5. From a commercial viewpoint, recovered reducing gases, e. g., carbon monoxide, hydrogen and hydrocarbon gases, can be utilized in various ways, for instance, as reducing atmospheres in heat treating furnaces or, preferably, as a supplementary supply of reducing gas for the present process. In addition, carbon dioxide can be recovered as a commercial by-product.

For instance, Fig. 5 shows that the partially-spent exhaust gases are drawn by means of a suitable pump through conduit 32 into a condenser 33 to remove the bulk of the water vapor. The gases from the pump outlet now containing hydrogen, carbon monoxide, hydrocarbons, carbon dioxide, and inert gases (mainly nitrogen) continue into the bottom of a carbon dioxide absorbing unit 34 of commercial design utilizing aqueous monoethanolamine solution as the absorbing agent. The carbon dioxide on passing upward through the absorbing unit with the reducing gases is removed by the downward-moving cold amine solution. The cold amine solution on leaving the bottom of the absorbing unit with its burden of carbon dioxide passes through a heat exchanger 35 to partially cool carbon dioxide-free amine solution that is then introduced at the top of the absorber unit. The carbon dioxide-containing amine solution leaving the unit is thereby preheated before its entry into the top of the amine solution reactivator 36. Heat introduced into this unit causes the amine solution to release the carbon dioxide which passes upward through a water cooler where vaporized and entrained amine solution is condensed and returned to the reactivator. Recovered carbon dioxide is withdrawn from the cooler as a valuable by-product. The hot amine solution, now free from carbon dioxide, is drawn off at the bottom of the reactivator by a pump and passed through the heat exchanger 35 where it is partially cooled, thereby heating the out-going carbon dioxide-containing amine solution from the absorber. The partially-cooled, carbon dioxide-free amine solution continues on from the heat exchanger to a water cooler 37 where it is cooled to the proper temperature for absorbing carbon dioxide and then returned to the absorber thus completing the absorption cycle. Reducing gases coming off the top of the absorber 34 contain hydrogen, carbon monoxide, hydrocarbons, and a small amount of inert gases, such as nitrogen, but are essentially free from carbon dioxide and water vapor. These reducing gases are available for reintroduction into the reduction muffle together with raw natural gas. Thus, the high concentrations of reducing components in the gas necessary to obtain maximum reduction of oxide at a rapid rate can be obtained with a minimum consumption of raw gas. The feed rate of oxide or, in other words, the furnace "throughput" capacity can thereby be markedly increased; and the heat requirements per unit weight of oxide reduced are considerably lowered since heat units, which other-

wise would be necessary to decompose large excesses of raw gas, are utilized instead for heating the oxide to the required reducing temperature.

By recovering and re-circulating unoxidized combustibles and hydrocarbons contained in the partially-spent exhaust gas, more complete utilization is made of the total reducing potential present in the original raw gas and, as a result, the actual amount of gas consumed per unit weight of oxide reduced more closely approaches the ideal or theoretical oxidation-reduction ratio of about one cubic foot of West Virginia natural gas per pound of oxide. In this manner, for any given feed rate, the percent total metal content obtained in the final reduced product is increased; and the consumption of gas per pound of oxide thus reduced is substantially lowered. The benefits derived from treating partially-spent exhaust gases to recover therefrom the active reducing components and re-circulating said recovered reducing components back through the reduction muffle are illustrated by the data presented in the following Table X. The data for test Nos. 44 to 48, inclusive, were obtained by re-circulating recovered reducing gases and the data for test Nos. 39 to 43, inclusive, were obtained by employing a large excess of raw natural gas only, e. g., 50% excess, to supply the concentration of reducing components necessary to obtain the required degree of reduction. The results shown in Table X were obtained in furnace A, the temperature being maintained in all cases at about 1800° F.

Table X

| Test No. | Feed Rate Oxide lbs./hr. | Reducing Gas, Ft. <sup>3</sup> /lb. Oxide | Recirculated Gas, Ft. <sup>3</sup> /lb. Oxide | Percent CO+H <sub>2</sub> in Recirculated Gas | Total Metal Content, percent Cu+Ni |
|----------|--------------------------|-------------------------------------------|-----------------------------------------------|-----------------------------------------------|------------------------------------|
| 39       | 64.8                     | 1.06                                      | —                                             | —                                             | 80.9                               |
| 40       | 38.1                     | 1.19                                      | —                                             | —                                             | 91.1                               |
| 41       | 52.6                     | 1.32                                      | —                                             | —                                             | 91.2                               |
| 42       | 65.8                     | 1.21                                      | —                                             | —                                             | 91.4                               |
| 43       | 55.0                     | 1.10                                      | —                                             | —                                             | 91.6                               |
| 44       | 39.8                     | 0.97                                      | 0.875                                         | *83.8                                         | 92.2                               |
| 45       | 78.2                     | 1.01                                      | 2.03                                          | N. D.                                         | 92.7                               |
| 46       | 72.6                     | 0.98                                      | 2.48                                          | *70.8                                         | 93.0                               |
| 47       | 41.8                     | 0.99                                      | 1.31                                          | N. D.                                         | 93.5                               |
| 48       | 58.5                     | 1.16                                      | 2.04                                          | *64.2                                         | 94.3                               |

N. D. = Not determined.

\* = Balance of re-circulated gas mainly hydrocarbons.

From an analysis of Table X, it can be seen that re-circulation of recovered reducing gases increases the degree of reduction obtained or alternatively, increases the production or "throughput" rate of reduced oxide of constant percentage reduction, whichever is desired. In general, this is true until re-circulation rates eventually are limited by muffle pressures, size of absorbing equipment, sensible heat losses, etc.

A small percentage of the partially-spent reducing gases can be allowed to escape from the charging bin to prevent excessive build-up of inert gases in the system. The sources of the inert gases are air occluded in the oxide charge and inert gases, such as nitrogen, present in the raw natural gas used for reduction. The quantity of valuable reducing components lost in this escaping gas is largely determined by the quantity of natural gas introduced into the muffle and the degree of reduction obtained. For example, on the assumption that 75% reduction is required, this theoretically would require about 0.75 cubic foot of gas per pound of oxide feed. Therefore, if

75% reduction is attained, any natural gas introduced into the muffle in excess of about 0.75 cubic foot per pound of oxide feed can be exhausted through the charging bin in the form of partially-spent reducing gases. The amount of excess natural gas introduced into the muffle is an amount sufficient only to prevent excessive build-up of inert gases in the recovered and recirculated reducing gases. Several methods exist of controlling bleeding of partially-spent exhaust gas through the charging bin to prevent excess build-up of the inert gas components in the muffle. The preferred method is the one hereinbefore described and is preferred largely on the basis of the simplicity of control which it provides. Increasing the input of natural gas above the theoretical value serves to increase considerably the heat requirements for the system, the excess heat being utilized primarily for decomposing the excess hydrocarbon gas which is exhausted from the muffle before its reducing potential has been profitably used. Therefore, for most economical production on a commercial scale, recovery and re-use of these reducing components in the partially-spent exhaust gas is a desirable, although not an essential, feature of the present invention, as shown by the data in the foregoing Table X. This is especially true where an outlet exists for the sale of the carbon dioxide recovered as a by-product.

Figs. 6 and 7 are sectional elevational views of a preferred structure of the novel, annular, oxide-reduction muffle of the present invention. In order to obtain the high degree of operating efficiency whereby high concentrations of uncontaminated reducing gases together with excellent heat-transfer characteristics are economically obtained, it is necessary to employ the present novel structure of reduction muffle. A preferred embodiment of the complete assembly of novel annular reduction muffle is illustrated in Fig. 6. The core-heating chamber, flame tube and annular oxide-reduction chamber portions of the annular muffle are shown in detail in Fig. 7. This novel structure is necessary to prevent excessive lowering of thermal efficiency when muffle diameters exceed about 5 inches. The example of the novel muffle structure illustrated in the aforementioned figures involves supplying heat to the core of the downward moving annular column of oxide as well as to the outside of said annular column of oxide. This is accomplished by providing an annular oxide-reduction chamber 20 (Fig. 7) for the downward passage of the oxide. The inside wall of the annular oxide-reducing chamber is common to the wall of the interior, closed-end, core-heating chamber 21 (Fig. 7), the heat being provided, for instance, either by a semi-long-flame burner or by a partial-premix burner inserted therein and comprising flame tube 22 (Fig. 7) and flame-retention tip 23 (Fig. 7). However, any type of burner may be used provided it satisfies the requirement of even, controlled distribution of heat. The outside wall of said annular oxide-reducing chamber is common to the interior wall of the exterior combustion muffle 24 (Fig. 6) to which heat is supplied preferably by tangentially-firing gas burners 25 (Fig. 6) arranged spirally relative to one another.

Control of the rate of combustion of the heating gases applied both externally and internally to the annular oxide-reducing chamber is effected by means known to those skilled in the art. Although heat can be supplied to the outside wall and to the core of the annular reduction cham-

ber from electric-power sources, e. g., electric-heating elements, it is preferable that the source of heat be obtained by the combustion of gas, oil or powdered fuels, more preferably by the combustion of the same natural gas which is introduced into the annular reduction chamber. Except in a very few areas where electric power is very cheap in comparison to the cost of gas, oil or coal, electric power is the least desirable source of heat for the oxide-reduction operation. A very important factor favoring employment of natural gas, oil and powdered coal as the source of heat is that the atmosphere produced by the combustion of these fuels, particularly natural gas, can be easily controlled to contain essentially no free oxygen, i. e., can be controlled to produce neutral to reducing atmospheres. This is of great importance in prolonging the service life of metallic muffles, particularly when operated at temperatures above about 1500° F. The muffle is preferably constructed of heat-resistant metal, more preferably a nickel-chrome-iron alloy sold under the trade-mark "Inconel."

After passage through the reducing chamber, the reduced oxide is cooled to at least below its reoxidation temperature in air, e. g., to at least about 550° F. Where the flow of gas is counter-current to the movement of oxide, this cooling of the reduced oxide to about 550° F. or lower is effected by the incoming, cold, raw, natural gas and also by water-cooled chamber 26 (Fig. 6) from whence it is discharged via a novel discharging mechanism 27 to bin 28 (Fig. 6). Where the flow of gas is concurrent with the movement of oxide, the cooling of the reduced oxide is almost solely effected by efficient heat transfer between water-cooled chamber 26 and the reduced oxide. Discharge mechanism 27 is the only continuously moving mechanical part in the entire novel reduction apparatus. This mechanism serves to regulate the rate of feed of the material through the apparatus but is not a gas-tight seal. In effect, the column of reduced oxide rests on a shelf or table within the discharger housing. The discharger blade, located well below the end of the muffle water jacket 26, gently pushes the reduced oxide off the shelf by a slow reciprocating motion. Since there is adequate space between the table-blade combination and the end of the muffle waterjacket, there is no shearing of the "ductile," reduced product; and consequently, wear of the moving blade is negligible. In other words, since this mechanism comes into contact only with reduced oxide of high metal content and not with unreduced oxide, it is not subjected to extremely high abrasive action of unreduced raw oxides. Furthermore, the carbon deposited on and within the reduced oxide particles serves as an excellent lubricant for the movement of both the blade and the reduced oxide across the surface of the table. As a result, this mechanism is relatively trouble-free in operation and has an unusually long service life.

The exact maximum temperature to which the reduced oxide must be cooled is influenced by the degree of activity of the reduced oxide. The gas-tight seals 29 and 30 (Fig. 6) at the receiving and discharging ports of bin 28, respectively, are so arranged that when one seal is open, the other is closed, thereby substantially excluding diluting and/or oxidizing agents, such as air, from the muffle. In employing counter-current flow of gas to oxide, the gas is introduced into the muffle through gas-inlet port 31 (Fig. 6).

In the present specification, where any total metal content values (per cent copper plus nickel) are given, these values represent analyses made on a carbon-free basis. Also, where the term nickel-copper oxide is employed, it is meant that said oxide is mainly a mixture of copper and nickel oxides although it is possible that compounds of copper oxide and nickel oxide, together with some iron oxide, silica, etc., might also be present.

It is to be observed that the present invention provides a novel process for producing metal from raw oxides, particularly nickel-containing oxides, which comprises reducing raw oxides of controlled particle size with hydrocarbon gases, particularly methane, to provide reduced oxide products having consistently uniform and high total metal contents and controllable, consistently uniform contents of highly-active carbon finely dispersed throughout the reduced oxide particles and then directly smelting and refining said reduced oxides without substantial additions of supplementary reducing agents. The foregoing novel process, when employed in the production of metal from raw oxides of said metal, results in the elimination of various complicated, expensive, time- and space-consuming operations necessary when producing metal from raw oxides by prior art methods and provides reduced oxides which are directly converted to metal by electric-arc or induction-furnace practice.

Furthermore, the invention provides a novel unitary reduction apparatus which combines the characteristics of excellent heat transfer between heat source, gases and oxide and high concentrations of uncontaminated reducing gases in contact with the oxides.

Moreover, the present invention provides a new product, heretofore unobtainable by conventional processes, which is a partially-reduced metallic oxide having a consistently high and uniform metal content and having a controlled, uniform, highly-active carbon content finely dispersed throughout the reduced oxide particles.

Although the present invention has been described in conjunction with certain preferred embodiments, it is to be understood that modifications and variations may be resorted to without departing from the spirit and scope of the invention, as those skilled in the art will readily understand. Thus, metallic oxides having oxygen dissociation pressures comparable to those of nickel oxide and copper oxide, including the oxides of lead, bismuth, cobalt, etc., can also be reduced by the present process regardless of whether or not nickel oxide and/or copper oxides are also present. However, cobalt oxide is the oxide most likely to be associated with nickel oxide and/or copper oxide and the present invention is particularly applicable to the treatment of the oxides of the metals cobalt, nickel and copper which have the atomic numbers 27, 28 and 29, respectively. Such variations and modifications are to be considered within the purview of the application and the scope of the appended claims.

We claim:

1. A process for controlled reduction of oxides of metal having atomic numbers from 27 to 29 to obtain partially-reduced oxide of consistently-uniform, high, total metal content and containing controlled amounts of uniformly dispersed, finely-divided, highly-active carbon and capable of being directly converted into high-quality metal without substantial additions of supple-

mentary reducing agents which comprises establishing a substantially vertical annular column of at least one of said oxides having a particle size between about 0.1 inch and about 0.5 inch, 5 said column having an effective width between about 2 inches and about 4 inches and having a ratio of surface area to volume of at least about 0.5; heating said oxide in a single operation to a temperature between about 1700° F. and about 10 1900° F. out of contact with combustion gases and in contact with countercurrently flowing hydrocarbon gas containing about 75% to about 95% methane to obtain controlled partial reduction of said oxide to a uniform total metal content between about 88% and about 95% and to obtain controlled uniform dispersion of about 0.4% to about 4.0% finely-divided, highly-active carbon within the particles of partially reduced oxide; and cooling said oxide in a non-oxidizing atmosphere to a temperature below at least about 20 550° F.

2. A process for controlled reduction of oxides of metal having atomic numbers from 27 to 29 to obtain partially-reduced oxide of consistently-uniform, high, total metal content and containing controlled amounts of uniformly-dispersed, 25 finely-divided, highly-active carbon and capable of being directly converted into high-quality metal without substantial additions of supplementary reducing agents which comprises establishing a substantially vertical annular column of at least one of said oxides having a particle size between about 0.04 inch and about 0.75 inch, said column having an effective width between 30 about 1 inch and about 5 inches and having a ratio of surface area to volume of at least about 0.4; heating said oxide in a single operation to a temperature between about 1500° F. and about 2000° F. out of contact with combustion gases and in contact with countercurrently flowing hydrocarbon gas to obtain controlled partial reduction of said oxide to a uniform total metal content of at least about 88% and to obtain controlled uniform dispersion of about 0.4% to about 35 4% finely-divided, highly-active carbon within the particles of the partially-reduced oxide; and cooling said oxide in a non-oxidizing atmosphere to a temperature below at least about 550° F.

3. A process for controlled reduction of oxides of metal having atomic numbers from 27 to 29 to obtain partially-reduced oxide of consistently-uniform, high, total metal content and containing controlled amounts of uniformly-dispersed, 40 finely-divided, highly-active carbon and capable of being directly converted into high-quality metal without substantial additions of supplementary reducing agents which comprises establishing a substantially vertical annular column of at least one of said oxides having a particle size between about 0.1 inch and about 0.5 inch, said column having an effective width between 45 about 2 inches and about 4 inches and having a ratio of surface area to volume of at least about 0.5; heating said oxide in a single operation to a temperature between about 1700° F. and about 1900° F. out of contact with combustion gases and in contact with concurrently flowing hydrocarbon gas containing about 75% to about 95% methane to obtain controlled partial reduction of said 50 oxide to a uniform total metal content of about 88% to about 95% and to obtain controlled uniform dispersion of about 0.05% to about 0.6% finely-divided, highly-active carbon within the 55 particles of the partially-reduced oxide; and

cooling said oxide in a non-oxidizing atmosphere to a temperature below at least about 550° F.

4. A process for controlled reduction of oxides of metal having atomic numbers from 27 to 29 to obtain partially-reduced oxide of consistently-uniform, high, total metal content and containing controlled amounts of uniformly-dispersed, finely-divided, highly-active carbon and capable of being directly converted into high-quality metal without substantial additions of supplementary reducing agents which comprises establishing a substantially vertical annular column of at least one of said oxides having a particle size between about 0.04 inch and about 0.75 inch, said column having an effective width between about 1 inch and about 5 inches and having a ratio of surface area to volume of at least about 0.4; heating said oxide in a single operation to a temperature between about 1500° F. and about 2000° F. out of contact with combustion gases and in contact with concurrently flowing hydrocarbon gas to obtain controlled partial reduction of said oxide to a uniform total metal content of at least about 88% and to obtain controlled uniform dispersion of about 0.05% to about 0.6% finely-divided, highly-active carbon within the particles of the partially-reduced oxide; and cooling said oxide in a non-oxidizing atmosphere to a temperature below at least about 550° F.

5. A process for controlled reduction of oxides of metal having atomic numbers from 27 to 29 to obtain partially-reduced oxide of consistently-uniform, high, total metal content and containing controlled amounts of uniformly-dispersed, finely-divided, highly-active carbon and capable of being directly converted into high-quality metal without substantial additions of supplementary reducing agents which comprises establishing a substantially vertical annular column of at least one of said oxides having a particle size between about 0.04 inch and about 0.75 inch, said column having an effective width between about 1 inch and about 5 inches and having a ratio of surface area to volume of at least about 0.4; heating said oxide in a single operation to a temperature between about 1500° F. and about 2000° F. out of contact with combustion gases and in contact with flowing hydrocarbon gas to obtain controlled partial reduction of said oxide to a uniform total metal content of at least about 88% and to obtain controlled uniform dispersion of about 0.05% to about 4.0% finely-divided, highly-active carbon within the particles of the partially-reduced oxide; and cooling said oxide in a non-oxidizing atmosphere to a temperature below at least about 550° F.

6. As a new article of manufacture, a partially-reduced particle of oxide of metal having atomic numbers from 27 to 29, said particle having a size of about 0.1 inch to about 0.5 inch and containing a total metal content of about 88% to about 95% together with about 0.4% to about 4.0% highly-active, finely-divided carbon uniformly dispersed within said partially-reduced particle.

7. As a new article of manufacture, a partially-reduced particle of oxide of metal having atomic numbers from 27 to 29, said particle having a size of about 0.1 inch to about 0.5 inch and containing a total metal content of about 88% to about 95% together with about 0.05% to about 0.6% highly-active, finely-divided carbon uniformly dispersed within said partially-reduced particle.

8. As a new article of manufacture, a partially-

reduced particle of oxide of metal having atomic numbers from 27 to 29, said particle having a size of about 0.04 inch to about 0.75 inch and containing a total metal content of at least about 88% together with about 0.05% to about 4.0% highly-active, finely-divided carbon uniformly dispersed within said partially-reduced particle.

9. As a new article of manufacture, a partially-reduced particle of oxide of metal having atomic numbers from 27 to 29, said particle having a size of about 0.04 inch to about 0.75 inch and containing a total metal content of at least about 88% together with about 0.4% to about 4.0% highly-active, finely-divided carbon uniformly dispersed within said partially-reduced particle.

10. As a new article of manufacture, a partially-reduced particle of a nickel-containing oxide, said particle having a size of about 0.04 inch to about 0.75 inch and containing a total metal content of at least about 88% together with about 0.4% to about 4.0% highly-active, finely-divided carbon uniformly dispersed within said partially-reduced particle.

11. A process for controlled reduction of a nickel-containing oxide to obtain partially-reduced oxide of consistently-uniform, high, total metal content and containing controlled amounts of uniformly dispersed, finely-divided, highly-active carbon and capable of being directly converted into high-quality metal without substantial additions of supplementary reducing agents which comprises establishing a substantially vertical annular column of said oxide having a particle size between about 0.1 inch and about 0.5

inch, said column having an effective width between about 2 inches and about 4 inches and having a ratio of surface area to volume of at least about 0.5; heating said oxide in a single operation to a temperature between about 1700° F. and about 1900° F. out of contact with combustion gases and in contact with counter-currently flowing hydrocarbon gas containing about 75% to about 95% methane to obtain controlled partial reduction of said oxide to a uniform total metal content between about 88% and about 95% and to obtain controlled uniform dispersion of about 0.4% to about 4.0% finely-divided, highly-active carbon within the particles of partially reduced oxide; and cooling said oxide in a non-oxidizing atmosphere to a temperature below at least about 550° F.

12. A process for controlled reduction of a nickel-containing oxide to obtain partially-reduced oxide of consistently-uniform, high, total metal content and containing controlled amounts of uniformly-dispersed, finely-divided, highly-active carbon and capable of being directly converted into high-quality metal without substantial additions of supplementary reducing agents which comprises establishing a substantially vertical annular column of said oxide having a particle size between about 0.04 inch and about 0.75 inch, said column having an effective width between about 1 inch and about 5 inches and having a ratio of surface area to volume of at least about 0.4; heating said oxide in a single operation to a temperature between about 1500° F. and about 2000° F. out of contact with combustion gases and in contact with counter-currently flowing hydrocarbon gas to obtain controlled partial reduction of said oxide to a uniform total metal content of at least about 88% and to obtain controlled uniform dispersion of finely-divided, highly-active carbon within the particles of the partially-reduced oxide; and

13. A partially-reduced particle of oxide of metal having atomic numbers from 27 to 29, said particle having a size of about 0.04 inch to about 0.75 inch and containing a total metal content of at least about 88% together with about 0.4% to about 4.0% highly-active, finely-divided carbon uniformly dispersed within said partially-reduced particle.

14. A partially-reduced particle of a nickel-containing oxide, said particle having a size of about 0.04 inch to about 0.75 inch and containing a total metal content of at least about 88% together with about 0.4% to about 4.0% highly-active, finely-divided carbon uniformly dispersed within said partially-reduced particle.

15. A partially-reduced particle of oxide of metal having atomic numbers from 27 to 29, said particle having a size of about 0.04 inch to about 0.75 inch and containing a total metal content of at least about 88% together with about 0.4% to about 4.0% highly-active, finely-divided carbon uniformly dispersed within said partially-reduced particle.

16. A partially-reduced particle of a nickel-containing oxide, said particle having a size of about 0.04 inch to about 0.75 inch and containing a total metal content of at least about 88% together with about 0.4% to about 4.0% highly-active, finely-divided carbon uniformly dispersed within said partially-reduced particle.

cooling said oxide in a non-oxidizing atmosphere to a temperature below at least about 550° F.

HARRY E. TSCHOP.

JOSEPH EDWIN CARTER.

CHARLES BRUCE GOODRICH.

References Cited in the file of this patent

UNITED STATES PATENTS

| Number    | Name  | Date            |
|-----------|-------|-----------------|
| 1,075,135 | Alton | Oct. 7, 1913 10 |

| Number    | Name            | Date           |
|-----------|-----------------|----------------|
| 1,480,212 | Lamothe         | Jan. 8, 1924   |
| 1,550,271 | Macklind et al. | Aug. 18, 1925  |
| 1,848,710 | Gustafsson      | Mar. 8, 1932   |
| 2,166,207 | Clark           | July 18, 1939  |
| 2,256,536 | Udy             | Sept. 23, 1941 |
| 2,296,841 | Gardner         | Sept. 29, 1942 |
| 2,302,615 | Linz            | Nov. 17, 1942  |
| 2,417,949 | Riveroll        | Mar. 25, 1947  |